

June 24, 1958

D. S. CHISHOLM ET AL

2,840,465

METHOD OF PRODUCING TITANIUM

Filed Oct. 20, 1952

3 Sheets-Sheet 1



Fig. 1

INVENTORS  
Douglas S. Chisholm  
Don F. Hall  
BY

Griswold & Gurdice  
ATTORNEYS

June 24, 1958

D. S. CHISHOLM ET AL

2,840,465

METHOD OF PRODUCING TITANIUM

Filed Oct. 20, 1952

3 Sheets-Sheet 2



June 24, 1958

D. S. CHISHOLM ET AL

2,840,465

METHOD OF PRODUCING TITANIUM

Filed Oct. 20, 1952

3 Sheets-Sheet 3



INVENTORS.  
Douglas S. Chisholm  
BY Don F. Hall

Griswold & Surdick  
ATTORNEYS

1

2,840,465

## METHOD OF PRODUCING TITANIUM

Douglas S. Chisholm and Don F. Hall, Midland, Mich., assignors to The Dow Chemical Company, Midland, Mich., a corporation of Delaware

Application October 20, 1952, Serial No. 315,604

6 Claims. (Cl. 75—84.5)

The invention relates to a method of and apparatus for the reduction of a metal halide vapor with magnesium. It more particularly concerns an improved method of and apparatus for the production of the metals, titanium and zirconium, by reacting a volatile halide thereof, especially the tetrachloride, with magnesium.

Heretofore in the reduction of titanium tetrachloride, for example, in accordance with the reaction:  $2\text{Mg} + \text{TiCl}_4 = \text{Ti} + 2\text{MgCl}_2$ , the magnesium used has been in the form of a pool of the molten metal in a retaining vessel with the upper surface of the pool exposed to the vapor of the titanium tetrachloride. In the ensuing reaction, there is formed a sponge-like mass of metallic titanium in situ, together with molten magnesium chloride as a by-product. A number of disadvantages inure to this practice which limits its usefulness. Among these disadvantages are that some of the magnesium becomes occluded in the titanium sponge and is thus prevented from being used, thereby lowering the efficiency of the reduction operation. The sponge so-formed in situ sticks to the walls of and tends to form a bridge in the retaining vessel and is difficult to remove, in spite of the fact that the magnesium metal during the reduction more or less floats upon molten magnesium chloride. Another disadvantage is that the reaction tends to get out of control allowing the magnesium to overheat and vaporize, thereby producing an undesirable flame-like reaction in which the magnesium burns as a vapor in the titanium tetrachloride vapor forming dust-like particles of metallic titanium instead of sponge. The dust-like particles of titanium thus produced are exceedingly difficult, if not impossible, to recover as massive titanium metal. Another disadvantage is that the titanium sponge is bulky and very reactive while hot necessitating essentially batchwise operation to permit cooling for the removal of the sponge from the retaining vessel and replacement of the supply of magnesium metal for the reduction. Similar difficulties arise in the reduction of zirconium tetrachloride with magnesium. Insofar as we are aware, there is neither a method nor an apparatus extant for the production of either titanium or zirconium metal by the reduction of the tetrachloride of these metals with magnesium which are not hampered in one way or another by the foregoing difficulties. Accordingly, it is the principal object of the invention to provide an improved method of and apparatus for carrying out the reduction of the aforesaid halides without the difficulties attendant upon the use of the conventional methods and means. Other objects and advantages will become apparent as the description of the invention proceeds.

Pursuant to the present invention, it has been discovered in reacting titanium tetrachloride vapor, for example with magnesium, that by particulating the magnesium and laying down a train or elongated pile of the magnesium particles upon a heat controlled supporting surface in an atmosphere of titanium tetrachloride

2

vapor, ignition and smoldering of the powder occurs in zones of the train intermediate its ends which move progressively and relatively slowly along the train away from the zone of formation as the particles are brought to ignition temperature. At the same time by abstracting sufficient of the resulting heat of the reducing reaction from the smoldering mass of magnesium particles through the supporting surface, they are prevented from bursting into flame and the reacting particles are maintained in a smoldering state until consumed. The particles of magnesium thus treated reach a temperature at least above that of the molten magnesium chloride formed in the reaction as a by-product, but the particles do not run together, instead they remain as a porous mass, thereby providing interstices throughout the pile. The titanium tetrachloride vapor is thereby enabled to permeate the pile and use all the magnesium particles, and much of the molten magnesium chloride is able to more or less drain away from the smoldering portion of the train as the reaction proceeds. As a result, there is formed in situ a titanium sponge occupying a space about twice that of the consumed train or pile of magnesium particles without producing titanium metal dust, the sponge being substantially free from unreacted magnesium metal. Moreover, the sponge so-produced may be readily removed from the supporting surface beyond the smoldering zone of the train without interrupting the reduction operation. The method is preferably carried out in continuous manner by continuously lengthening the train or pile of magnesium particles at one end ahead of the smoldering portion, at a rate sufficient to keep a supply of magnesium particles ahead of the smoldering ones, while removing the produced sponge from the other end behind the smoldering portion. Analogous results are obtained on applying the same method with zirconium tetrachloride vapor. The invention then consists of the improved method and apparatus herein fully described and particularly pointed out in the claims, the annexed drawing and following description setting forth various modes of practicing the invention.

In the said annexed drawing, Fig. 1 is a schematic diagram illustrating the method of the invention together with apparatus for practicing the same.

Fig. 2 is a side elevation largely in section of an apparatus according to the invention.

Fig. 3 is a horizontal section of the apparatus on the line 3—3 of Fig. 2.

On referring to Fig. 1, it will be apparent that this is a diagrammatic representation of the method generally outlined above and the figure illustrates the principle of carrying out the reaction in accordance with the invention, as applied to the production of titanium, for example, by a controlled smoldering of a train or pile of particles of magnesium in an atmosphere of titanium tetrachloride vapor. In this figure is shown a supporting surface 1, on which the reaction of the magnesium particles with the halide vapor is to take place. The supporting surface is provided with temperature control means comprising a set of pipes 2, embedded in the supporting surface, through which air at a suitable temperature may be passed. The supporting surface is placed within an envelope, not shown, for retaining an ambient atmosphere 3 of titanium tetrachloride vapor with which the magnesium particles are to react. Means are provided, such as the particle feeder 4, above the supporting surface for depositing thereupon the magnesium particles, the rate of deposition being subject to control, as by means of the valve 5.

With this apparatus, a train of particulated magnesium is shown as having been deposited upon the supporting

surface by a relative sideways movement of the feeder outlet 6 with respect to the supporting surface in the direction of left to right. The train of particles so-formed passes through a number of changes occurring in sequence in more or less distinct zones moving along the train in the ensuing reaction which consumes the train as it forms leaving titanium sponge in situ.

As to these changes, the train begins, as aforesaid, with the deposition of the particles on the supporting surface. This takes place at the pile- or train-forming zone 7 below the feed pipe 6 from which the particles fall. The particles at this stage are relatively cold; that is the temperature is below that at which they will spontaneously ignite in the tetrachloride atmosphere. The pile-forming zone is followed by a preheating zone 8 in which the particles are subjected to heating both by contact with the supporting surface and by contact with adjacent particles already ignited and burning in the following zone. The heating which occurs in the preheating zone raises the temperature of the particles progressively along the preheating zone to a temperature at which ignition or burning of the magnesium particles in the halide atmosphere begins. Thus, an ignition zone is established adjacent to the hotter end of the preheating zone, as indicated by numeral 8, the hotter end being remote from the zone of formation. The ignition zone on the forward end is sharply distinct from the preheating zone while the rear of the ignition zone merges into a smoldering zone designated by numeral 10 where the particles become hotter as the reaction proceeds. In the front of the smoldering zone, the ignited particles communicate some of their heat to adjacent unignited particles and as already mentioned thereby maintain ignition in the ignition zone. Burning of the particles continues in the smoldering zone until all magnesium particles are consumed forming titanium sponge in situ as a loaf or cake and molten magnesium chloride.

In the smoldering zone, more than enough heat is liberated to maintain the reaction at a smoldering pace, and, accordingly, in this zone, the smoldering particles are subjected to a heat exchange in which a sufficient amount of the heat of the reaction is abstracted from the pile as through the supporting surface, by means of a cooling air blast through pipes 2, to prevent the smoldering particles from overheating and bursting into flame. The amount of heat exchange required to maintain the burning of the ignited particles at a smoldering pace is readily ascertained by trial as by watching the smoldering zone and suppressing the reaction by cooling the supporting surface enough to prevent flame formation. It has been found by maintaining the supporting surface under the smoldering zone at a temperature sufficient to cause ignition of the particles in the halide atmosphere but not in excess of about 900° to 950° C. The reaction rate can be maintained at a smoldering pace. A preferable temperature for the supporting surface is above that sufficient to maintain the by-product magnesium chloride in the molten state (e. g. about 708° C.) but less than about 850° C. Temperatures lower than the melting point of magnesium chloride can be used (e. g. 600° C.) if the solid magnesium chloride which then tends to collect upon the supporting surface can be removed.

Both during and for some time after the smoldering action, a substantial proportion of the magnesium chloride drains out of the sponge. The zone of such drainage of the train is indicated at 11 and partially overlaps the smoldering zone 10. The resulting partially drained sponge 12 left at the end of the smoldering zone, after all the magnesium has been consumed in reducing tetrachloride vapor, may be removed from the supporting surface, as by a cooled scraper 13, in the form of chunks of sponge 14.

The by-product magnesium chloride which in part drains out of the sponge and off the supporting surface, 1

as shown, may be collected in any convenient manner below the supporting surface, and, if desired, reworked for its magnesium content in conventional manner for reuse in the method.

5 The foregoing method may be conducted advantageously upon a moving hearth or supporting surface which moves sideways away from the train-forming zone beneath the magnesium particle feeder at a rate which is equal, on the average, to the rate at which the zone of ignition moves toward the forming end of the train. In this way, the various zones above described in connection with Fig. 1 are obtained which remain in the same relative positions and the process is thereby made continuous. In such mode of operation, the path of the train of magnesium particles is preferably made in the form of a segment of a circle as by the use of a revolving supporting surface arranged beneath a magnesium particle feeder which remains stationary with respect to the supporting surface on which the feeder deposits the particles as the surface moves.

20 This mode of operation and an apparatus therefor is illustrated in Figs. 2 and 3 which will now be described. In this mode of operation, the supporting surface for the magnesium particles may be in the form of a hollow air cooled disc 15, for example, secured to the lower end of the hollow drive shaft 16, the disc being within the reaction vessel 17 which holds the atmosphere containing the titanium tetrachloride vapor to be reduced. The reaction vessel 17 is supported in a furnace setting 18 by means of which the disc 15 may be heated to a temperature sufficient at least to initiate the reaction of the magnesium with the halide vapor to be reduced and preferably to maintain the by-product magnesium chloride in the molten state. The reaction vessel 17 is provided with a gas tight cover 19 for retaining within the vessel the atmosphere containing the halide vapor with which the magnesium is to react. The cover is provided with an opening 20 through which passes the aforesaid shaft 16. The stuffing box 21, secured to the cover around the opening 20, provides a gas tight seal for the shaft 16. The shaft is supported near its upper end by means of the thrust-bearing 22 which rests on support 23. Drive pulley 24 is secured to the upper end of the shaft and is driven by means of motor 25 through the reduction gearing 26, pulley 27, and belt 28. 25 Through the hollow shaft 15 extends the pipe 29 for conveying cooling air to the inside 30 of the disc 15. The lower end of the pipe 29 carries a pipe T31 for facilitating the distribution of the cooling air within the hollow disc. The upper end of the pipe extends through the supporting bracket 32 to a source of air, not shown. The return air from the hollow disc escapes up the annular space 33 between the outside of pipe 29 and the inside of the hollow shaft 16.

30 The particulated magnesium to be deposited upon the disc 15 is introduced into the vessel from a supply hopper 34 through a screw conveyor 35 and feed pipe 36, the outlet 37 of which is arranged directly over the disc 15 a short distance inward of its periphery. Receptacle 38 holds a supply of the halide (e. g. liquid titanium tetrachloride) which is vaporized in the vessel 17 and reduced to metal on the disc 15. The receptacle 38 is connected to the inside of the reaction vessel through the cover by pipe 39 having a valve 40 for controlling the rate of introduction of the halide into the vessel. A manometer 41 provides a means for ascertaining the difference in the pressure between the atmosphere outside the vessel and that on the inside. Extending through the cover 19 at an oblique angle is a viewing device consisting of a tube 42 with a transparent eye-piece 43 through which may be seen the upper side of the hollow disc 15. The reaction vessel 17 is provided with a hopper bottom 44 on the inside of which is arranged the inclined screw conveyor 45. As shown, the screw conveyor comprises the single plate helix 46 wound on the shaft 47, the helix having small openings 48 therethrough to allow liquid to drain so that

the conveyor will not function to elevate liquid. The lower end of the shaft 47 is journaled in the bearing 49 mounted in the vessel. The upper end of the conveyor extends into an inclined tube 50 which passes through the vessel to the outside. The lower end 51 of the inclined tube extends into the vessel for a sufficient distance to form a seal with the pool 52 of molten magnesium chloride which is maintained in the vessel during operation. The vessel is provided with an outlet 53 below the surface 54 of the pool of molten magnesium chloride, the outlet being provided with a trap 55 by means of which the level of the surface 54 is maintained above the lower end 51 of the inclined pipe. The trap has an outlet 56 outside the furnace setting through which molten magnesium chloride is withdrawn from the pool. The upper end of the inclined pipe is provided with a flange 57 to which is secured the cover plate 58. The cover plate is provided with an opening 59 which forms a bearing for the upper end of the screw conveyor shaft 47. Near the upper end of the inclined tube 50 is a downwardly extending T, 60, having a flanged opening 61 to which may be detachably secured the vessel 62 by means of clamps 63.

An air cooled scraper indicated generally by numeral 64 (Fig. 3) is provided over the disc 15 for removing the metal sponge formed thereon. As shown, this device comprises a hollow scraper head 65 carried on one end of a hollow shaft 66 by means of which the head 65 is moved back and forth across the upper surface of the disc 15 as indicated in dotted outline. The shaft 66 extends through a tube 67 one end of which is joined to the side of the vessel 17, around an opening 68 therein, and the other extends through the side of the furnace setting 18. A stuffing box 69 is provided on the outer end of the tube 67 for making a seal around the shaft 66, the seal permitting longitudinal reciprocatory movement without leakage of air into the vessel 17. A bearing in the form of an annular ring 70, together with the stuffing box 69, maintains the shaft 66 aligned in the bore of tube 67. Reciprocatory motion of the shaft 66 is provided through the link 71 connecting the shaft with the crank pin 72 on gear wheel 73 which is rotated by pinion 74 on motor 75.

Cooling of the scraper head 65 is effected by means of the pipe 76 which extends through shaft 66 to near the inside of the working face 77 of the scraper head. The pipe 76 is connected by a flexible hose 78 to a source of air (not shown). The air delivered by the pipe 76 to the scraper head exhausts through the annular space 79 between the inside of the shaft 66 and the outside of the pipe 76.

In operation, as with titanium tetrachloride for example, the reaction vessel is maintained at a temperature sufficient to maintain the pool 52 of magnesium chloride in the molten state, the molten magnesium chloride of the pool forming a seal against the escape of tetrachloride vapor from the reaction vessel through the outlet 53 and the tube 50. The tetrachloride to be reduced is introduced into the reaction vessel at a rate preferably sufficient to maintain therein a slightly greater pressure of the halide vapor than the atmospheric pressure outside the vessel. In starting up, the heating of the vessel by the furnace setting 18 in time heats the hollow disc 15 until it is hot enough to initiate the reducing reaction between particulated magnesium and the tetrachloride vapor. When the disc is thus made sufficiently hot feeding thereon of the train of particulated magnesium is begun. This is accomplished by revolving the disc 15 slowly by starting motor 25 and operating the screw conveyor 35 so as to convey magnesium particles from the supply hopper 34 to the upper surface of the disc 15. While magnesium particles are allowed to fall from the outlet 37 onto the slowly moving disc 15, a train of particles is thereby laid down as indicated at 80. As already explained in connection with Fig. 1, that by the formation of the train of magnesium particles upon a heated supporting surface in the tetrachloride atmosphere, there is established in the train a

number of more or less distinct zones of action which characterize the method. With the apparatus of Figs. 2 and 3, a series of zones similar to that of Fig. 1 is formed but in a train having the form of a segment of a circle instead of a straight line since the train is deposited upon a revolving surface from a fixed feeding point. Referring to Fig. 3 in particular, these zones are indicated as follows: pile or train-forming zone, 81; preheating zone, 82; ignition zone, 83; smoldering zone, 84; drainage zone, 85; sponge removal zone, 86. The depth of the pile or train is controlled by the rate of actuation of the screw conveyor 35 as well as by the rate of turning of the disc 15. The depth of the train which gives satisfactory burning or smoldering does not appear to be sharply critical. If the train is relatively thin propagation of the smoldering zone into the preheating zone is more or less erratic and discontinuity of operation may result. If the train depth is excessive, there is a tendency for some magnesium particles to be left unburned. Proper depths for the train are readily ascertained by trial during operation and are evidenced by continuity of the burning or reaction of the magnesium in the tetrachloride vapor without flame, and the absence of unconsumed magnesium particles in the resulting sponge. Successful operation has been had, for example, at depths ranging from  $\frac{1}{4}$  inch to as much as  $1\frac{1}{2}$  inches.

In any event, the rate of turning of the disc must not exceed the rate at which the ignition zone 82 progresses along the train which becomes heated, then ignites, and smolders in zones progressing along the train as indicated in the drawing. It will be understood that the lengths of the zones is not critical and varies with operating conditions, and sufficient time should be allowed in generating the train for the smoldering to be completed before removing the sponge from the disc. By directing the viewing tube at the point in the train where the ignition zone merges into the preheating zone, the rate of turning of the disc can be adjusted readily to that which will maintain the ignition zone close to the pile- or train-forming zone 81.

As smoldering proceeds, the temperature of the smoldering portion of the train tends to rise rapidly and the temperature of the hollow disc 15 is to be controlled and limited by directing a cooling air blast into it through pipe 78 in amount sufficient to maintain the reaction of the pile of particles at a smoldering pace as shown by the absence of flame. The rate at which the zone of ignition proceeds along the train of preheated particles, when the desired smoldering conditions are reached and operation is continuous, is for example from about 0.1 to 0.5 foot per minute for particles passing through a No. 20 sieve with 95 percent retention on a No. 200 sieve and laid in a train containing per lineal foot from 1 to 36 grams of magnesium. For example, a disc, 20 inches in diameter on which is formed a pile of magnesium particles in the form of a segment of a circle about 2 inches wide and about  $2\frac{1}{2}$  inches from the periphery of the disc, may be turned at the rate of about 0.2 to 0.6 R. P. M. depending upon the rate of smoldering. The smoldering zone thus moves along the sequential train on the disc in a direction opposite to that in which the disc rotates, and, by a suitable regulation of the speed of rotation of the disc, is maintained constantly at about the same position with respect to the outlet 37 during operation. The by-product magnesium chloride in part drains out of the resulting sponge in the drainage zone 85 and drips off the disc into the pool 52 while the disc turns.

The partially drained sponge left after the smoldering has ceased is periodically pushed or scraped off the disc in chunks by the cooled scraper head 65, which is caused to reciprocate back and forth across the path of the train by actuating motor 75, the head being cooled sufficiently to prevent the sponge from sticking to it by directing air into the head through the hose 78. With this scraper device, the sponge is somewhat compacted on be-

ing subjected to the pressure of the scraper head as it pushes against the sponge in scraping it off the disc, as the sponge is at a temperature generally above 708° C., the melting point of magnesium chloride, and somewhat plastic at this stage. The resulting more or less compacted hot chunks or pieces of sponge fall into the pool 52 of molten magnesium chloride and on actuating the screw conveyor 45 are carried out of the pool through a seal of magnesium chloride in tube 50 into the vessel 62 out of contact with air. After sufficiently cooling the chunks in the vessel, it may be removed from the conveyor and emptied. Much of the by-product magnesium chloride overflows through the trap 55 and is discharged at 56, the balance of the magnesium chloride is contained in the pores of the sponge.

The titanium sponge thus produced is readily worked into massive metal by conventional methods to yield a high quality metal.

In providing the particulated magnesium for use in the method, it is desirable to eliminate particles which are dust-like from the feed, although a small amount, such as up to 5 percent by weight, of dust-like particles can be tolerated. In general, it is desirable to use particles larger than those passing through a No. 200 sieve (of the standard screen scale) to avoid loss by dusting. A relatively short drop, such as 6 inches, from the outlet 37 of the feed pipe to the supporting surface is desirable as the short drop tends to lessen dusting and also undesirable bouncing and rolling of the particles on reaching the supporting surface. Large particles are objectionable because on melting they coalesce into still larger molten masses which tend to flow off the reaction supporting surface without forming the sequence of zones described. Particles between these extremes may be used and may be produced in various known ways, such as by grinding, chipping, milling, and atomizing. Particles which are more or less equiaxed, such as those made by the usual atomizing methods, produce the best results. Equiaxed particles as large as those passing through a No. 10 sieve may be used, although somewhat finer particles are preferable, such as those passing through a No. 20 sieve with at least 95 percent retention on a No. 200 sieve.

The particles of magnesium as introduced into the tetrachloride atmosphere, on being caught upon the supporting surface for reaction, are relatively cold so that reaction does not commence to a significant extent until the particles are actually in the form of a pile or train upon the supporting surface. This mode of operation overcomes the clogging at the outlet 37 which can occur when the particles fed through it are too hot or too fine and tend to burn as they fall through the pipe 36. If desired, an inert gas, such as argon or helium, may be fed into the pipe 36 as though a pipe connection 64 to block the tendency for the vapor of the volatile halide to enter the pipe 36 from the reaction vessel 17. The dilution, if any, which may result from the presence of the inert gas in the atmosphere in the reaction vessel does not significantly affect the reduction reaction, although provision for venting the inert gas from the reaction vessel may be required as by means of a vented condenser, not shown.

The particles of magnesium may be deposited upon the hearth or supporting surface at as rapid a rate as that at which the zone of ignition advances in the resulting train or elongated pile. At the same time, the halide to be reduced is introduced into the reaction vessel at a rate sufficient to maintain therein a pressure of the halide vapor preferably in excess of the atmospheric pressure outside the vessel. For example, the vapor pressure in the reaction vessel of the halide to be reduced may exceed the atmospheric pressure by 1 to 20 inches of water (as in manometer 41) but other pressures may be used.

While the invention has been exemplified with particular reference to the deposition of the train or pile of particulated magnesium upon flat surfaces, it is to be understood that other solid supporting surfaces may be used in

similar manner, although not flat, such as cylindrical or conical surfaces. In such instances, the cylinder or cone, for example, is arranged to revolve on its axis in such a manner that the underside of a more or less horizontal plain surface will be tangent to the revolving surface at least at the place where the particles are deposited. It will be found also that even though the supporting surface is made to slope away from the point of deposition of the particles so as to facilitate drainage of the by-product magnesium chloride, the tendency for the particles to roll off is reduced, if not completely counteracted, during their reaction with the halide vapor, the reaction products of which give adhesion to the particles for each other and the supporting surface when wet with molten magnesium chloride.

Among the advantages of the invention are that the magnesium, in particulate form and arranged in a pile and made to smolder, becomes completely consumed in the atmosphere of the halide to be reduced. There is, therefore, a maximum efficiency of use of the magnesium. The metal obtained from the reduced halide vapor is substantially all in the form of easily recoverable sponge, there being substantially no produced metal in the form of dust-like particles which are difficult, if not impossible, to recover. The method is adapted to continuous operation without contamination of the metal product by the atmosphere. The reduction operation is subject to easy accurate control by regulation of the input of particulated magnesium metal and removal of reaction heat. The magnesium is not fed onto an already reacting body of magnesium instead the magnesium reacts with the halide vapor without hindrance from the magnesium supply for the reaction because the pile or train of magnesium particles used in the reduction is formed in the reaction zone before the reaction occurs. The reaction is confined to the surfaces of the particles of magnesium in the pile or train; hence the walls of the reaction vessel enclosing the halide vapor to be reduced do not become fouled up with metal reduced from the halide. The reaction of the magnesium with the halide vapor can be carried out upon horizontal or sloping surfaces without confining sidewalls because the magnesium is in particulate form and the particles neither run together nor off the surfaces.

We claim:

1. The method of producing titanium sponge by reacting magnesium with titanium tetrachloride which comprises depositing upon a supporting surface in an atmosphere containing titanium tetrachloride vapor a pile of magnesium in particulate form, said surface having a temperature above the melting point of magnesium chloride whereby the magnesium particles burn in the titanium tetrachloride vapor forming titanium sponge in situ and molten magnesium chloride; removing heat from the burning pile at a rate sufficient to maintain the burning at a smoldering pace; and draining molten magnesium chloride from the pile as it smolders.

2. The method of producing titanium sponge by reacting magnesium with titanium tetrachloride which comprises depositing upon a supporting surface in an atmosphere containing titanium tetrachloride vapor a pile of magnesium in particulate form, said surfaces having a temperature above the melting point of magnesium chloride whereby the magnesium particles burn in the titanium tetrachloride vapor forming titanium sponge in situ and molten magnesium chloride; removing heat from the burning pile at a rate sufficient to maintain the burning at a smoldering pace; draining molten magnesium chloride from the pile as it smolders; and removing the resulting titanium sponge from the supporting surface.

3. The method of reacting magnesium with titanium tetrachloride vapor which comprises catching a falling stream of particulated magnesium on a heat-absorbing surface moving in a direction sideways of the stream so as to form an elongated shallow pile of particulated magnesium on the said surface, said falling stream of par-

particulated magnesium having a temperature below that at which the particles spontaneously ignite in titanium tetrachloride vapor while providing the pile with an ambient atmosphere comprising titanium tetrachloride vapor; maintaining the said heat-absorbing surface at a temperature of at least 708° C., whereby the portion of the pile remote from the point receiving the falling stream becomes heated and smolders on the said surface in the said atmosphere producing molten titanium sponge in situ and molten magnesium chloride, a portion of said molten magnesium chloride dripping off the heat-absorbing surface as the particles smolder, the smoldering progressing along the pile toward the point of formation; removing heat from the smoldering portion of the pile through the said heat-absorbing surface at a rate sufficient to prevent the smoldering portion of the pile from bursting into flame, the rate of sideways movement of the heat-absorbing surface being equal to the average rate of progression of the smoldering along the pile; and removing from the heat-absorbing surface the so-formed titanium sponge beyond the smoldering portion.

4. The method of producing titanium sponge by reacting magnesium with titanium tetrachloride which comprises depositing upon a supporting surface in an atmosphere containing titanium tetrachloride vapor a pile of magnesium in particulate form, said surface having a temperature above the melting point of magnesium chloride whereby the magnesium particles burn in the titanium tetrachloride vapor forming titanium sponge in situ and molten magnesium chloride, a portion of said molten magnesium chloride dripping off the supporting surface as the magnesium particles burn; removing heat from the burning pile at a rate sufficient to maintain the burning at a smoldering pace; collecting in a pool the magnesium chloride which drips off the supporting surface; and withdrawing the so-produced titanium sponge from the reaction zone through the said pool.

5. The method of producing titanium sponge by reacting magnesium with titanium tetrachloride which comprises forming an atmosphere containing titanium tetrachloride vapor in a reaction zone; depositing upon a heat-absorbing surface in the said zone above the bottom thereof a pile of magnesium in solid particulate form, said surface having a temperature above the melting point of magnesium chloride, whereby the magnesium particles burn in the said atmosphere forming titanium sponge in situ and molten magnesium chloride, a portion of said molten magnesium chloride dripping off the heat-absorbing surface as the magnesium particles burn; removing heat from the burning pile at a rate sufficient to maintain the burning at a smoldering pace; collecting in a pool below the heat-absorbing surface the portion of the magnesium chloride which drips off the heat-absorbing surface; and scrap-

ing the titanium sponge so-formed off the heat-absorbing surface into the said pool.

6. The method of reacting magnesium with titanium tetrachloride vapor which comprises catching a falling stream of particulated magnesium on a heat-absorbing surface moving in a direction sideways of the stream so as to form an elongated shallow pile of particulated magnesium on the said surface, said falling stream of particulated magnesium having a temperature below that at which the particles spontaneously ignite in titanium tetrachloride vapor while providing the pile with an ambient atmosphere comprising titanium tetrachloride vapor; maintaining the said heat-absorbing surface at a temperature of at least 708° C., whereby the portion of the pile remote from the point receiving the falling stream becomes heated and smolders on the said surface in the said atmosphere producing titanium sponge in situ and molten magnesium chloride, a portion of said molten magnesium chloride dripping off the heat-absorbing surface as the particles smolder, the smoldering progressing along the pile toward the point of formation; removing heat from the smoldering portion of the pile through the said heat-absorbing surface at a rate sufficient to prevent the smoldering portion of the pile from bursting into flame, the rate of sideways movement of the heat-absorbing surface being equal to the average rate of progression of the smoldering along the pile; collecting in a pool below the heat-absorbing surface the magnesium chloride which drips off the heat-absorbing surface; and removing from the heat-absorbing surface the so-formed titanium sponge beyond the smoldering portion.

#### References Cited in the file of this patent

##### UNITED STATES PATENTS

|    |           |                 |                |
|----|-----------|-----------------|----------------|
| 35 | 1,321,684 | Turner          | Nov. 11, 1919  |
|    | 1,373,038 | Weber           | Mar. 29, 1921  |
|    | 1,558,965 | Clevenger       | Oct. 27, 1925  |
|    | 2,205,854 | Kroll           | June 25, 1940  |
|    | 2,564,337 | Maddex          | Aug. 14, 1951  |
| 40 | 2,567,838 | Blue            | Sept. 11, 1951 |
|    | 2,586,134 | Winter          | Feb. 19, 1952  |
|    | 2,607,674 | Winter          | Aug. 19, 1952  |
|    | 2,663,634 | Stoddard et al. | Dec. 22, 1953  |
|    | 2,763,542 | Winter          | Sept. 18, 1956 |
| 45 | 2,766,113 | Chisholm et al. | Oct. 9, 1956   |

##### FOREIGN PATENTS

|            |               |               |
|------------|---------------|---------------|
| 386,621    | Great Britain | Feb. 16, 1933 |
| 832,205    | Germany       | Feb. 21, 1952 |
| 50 686,845 | Great Britain | Feb. 4, 1953  |

##### OTHER REFERENCES

Metal Powder Report, vol. 7, No. 4, December 1952,  
page 50.